

# UNITED STATES PATENT OFFICE.

PETER S. BRAUCHER, OF READING, PENNSYLVANIA.

## SOFT-METAL ALLOY.

1,304,849.

Specification of Letters Patent. Patented May 27, 1919.

No Drawing.

Application filed February 4, 1919. Serial No. 274,992.

*To all whom it may concern:*

Be it known that I, PETER S. BRAUCHER, a citizen of the United States, residing at Reading, in the county of Berks and State 5 of Pennsylvania, have invented certain new and useful Improvements in Soft-Metal Alloys, of which the following is a specification.

This invention relates to improvements 10 in soft metal alloys and the object in the present instance is to provide an improved alloy suitable for use as a soft metal bearing metal, one in which the cost is maintained at approximately the minimum, and 15 in which the desired toughness is obtained without that brittle hardness that so often accompanies the effort at toughness.

A further object is to provide, in the composition, an element that will act as a 20 cleansing agent or scavenger, so that whatever grit there may be contained in the mixture, will be absorbed or nullified.

The distinguishing feature of my present invention therefore is the presence of phosphorus, which is added to the other constituents of the alloy before melting, or 25 while in a molten state.

The addition of phosphorus to the ordinary constituents of a soft metal bearing 30 metal will toughen the resultant product, remove all tendency to grit, and as a consequence, result in better lubrication with ordinary lubricants, thus reducing very materially the tendency to overheated bear- 35 ings.

An important practical advantage of the present invention when used in connection 40 with the ordinary type of soft bearing metal comprising as its principal constituents, lead, tin and antimony, is that its use permits of the formation of a satisfactory bearing metal containing less of the relatively high priced toughening elements, tin and antimony, and more of the low priced 45 lead element than would otherwise be required.

The addition of the phosphorus content to the bearing metal not only toughens the metal but tends to neutralize the foreign

substances and grit, which admittedly aids 50 materially in the lubrication obtained with any given lubricant.

It has been definitely determined that the phosphorus content will cause a more 55 satisfactory fusing of the metal than could be effected, for instance, by the use of caustic soda in its stead, while at the same time the phosphorus acts as a scavenger in cleansing up the metal and neutralizing the foreign particles that would otherwise tend 60 to grit.

The proportionate amount of phosphorus as well as the character of some of the other constituents used, may vary, while the characteristic advantages obtained by the use 65 of phosphorus will still obtain.

My present invention contemplates an alloy formed of lead, tin, antimony and phosphorus in substantially the following proportions:—

|            |           |
|------------|-----------|
| Lead       | 89 parts. |
| Tin        | 7½ parts. |
| Antimony   | 3½ parts. |
| Phosphorus | 0½ parts. |

70

75

The above named constituents may be mixed together before melting, but I prefer to form a molten mixture of the tin and antimony, add thereto a portion of the phosphorus to be used, then add the product thus obtained to molten lead and then, to the last named mixture, add the remainder of the phosphorus to be used.

It has been determined that in the resultant product, there is sufficient to warrant 85 the belief that the phosphorus is present as metallic phosphorus held in solidified solution of lead, antimony and tin, but whether this is correct or not, the actual practical improvement accomplished in soft bearing 90 metals by the use of my present invention has been positively established by actual use over a comparatively long period of time.

What I claim as my invention is:—

1. A soft metal alloy containing eighty-nine per cent. of lead and one-quarter of one per cent. of phosphorus.
2. A soft metal alloy containing eighty-

nine per cent. of lead, one-quarter of one per cent. of phosphorus and the remainder composed of tin and antimony.

3. A soft metal alloy containing eighty-nine per cent. of lead, one-quarter of one per cent. of phosphorus and the remainder of tin and antimony in the proportions of two parts of tin to one part of antimony.

4. An alloy consisting of eighty-nine parts lead, seven and one-half parts tin, three and one-quarter parts antimony, and 10 one-quarter of one part phosphorus.

In testimony whereof I affix my signature.

PETER S. BRAUCHER.